# EUROPEAN PATENT SPECIFICATION

(11) **EP 0 118 898 B1**
(45) Date of publication and mention of the grant of the patent: **26.10.1988**
(21) Application number: 84102578.6
(22) Date of filing: 09.03.1984
(51) Int. Cl.: A41D 31/00, A41D 13/10, A41D 13/00

(54) **Protective garment**
Schutzkleidung
Vêtement protecteur

(30) Priority: 11.03.1983 US 474466
(43) Date of publication of application: 19.09.1984
(73) Proprietor: BETTCHER INDUSTRIES, INC., Birmingham Ohio 44816 (US)
(72) Inventor: Bettcher, William H., Vermilion Ohio 44089 (US); Bettcher, Laurence A., Huron Ohio 44839 (US)
(74) Representative: Baillie, Iain Cameron

(56) References cited:
- DE-A- 1 610 495
- DE-A- 2 336 200
- DE-A- 3 023 990
- FR-A- 2 366 810
- GB-A- 2 018 323
- US-A- 4 004 295

## Description

The invention relates to protective garments made of wire and fiber strands and an elastomeric coating.

Cut-resistant garments have been proposed of steel wire and aramid fiber. A cut-resistant knitted glove has been made of yarn having a core of two stainless steel strands and a strand of aramid fiber, overwrappred in opposite directions with aramid fiber strands or with an aramid strand and a covering strand of nylon (polyamide) (see GB-A-2 018 323). Aramid fiber is strong and cut-resistant, and such a glove is extremely effective and useful in protecting against injury from sharp products or tools, e.g., in cutting and processing meat products; yet, the aramid yarn is somewhat abrasive (self abrasive, causing wear, and also abrasive or harsh to the feel), tends to absorb dirt, fat, blood or other fluids, and is not as easily cleaned as might be desired. Moreover, detergents, light and water tend to break down aramid fiber. In addition, aramid fiber, which accounts for much of the strength and cut-resistance of the glove, is relatively expensive. Utilizing a covering nylon strand in forming the yarn diminishes the above disadvantages, but greater improvement is still desired. For example, such a glove still is not liquid or moisture proof, slip resistant or heat resistant. Due to one or a combination of these shortcomings, the market for the present gloves is limited. The glove industry, in particular, has long sought a satisfactory liquid-proof cut and heat-resistant glove that is light-weight, comfortable and reasonably priced. Where protective gloves have been knit from bare steel wire, such as the "chain-mail" type of DE-A-30 23 990, it has been proposed to protect the wearer's hand from the harsh metal by coating the chain mail with elastomeric material.

The present invention provides a high strength, flexible, relatively light-weight garment of substantially improved cut-resistance, that is moisture and oil resistant, nonabsorbent, slip resistant, durable, comfortable to wear and use, and economical to manufacture.

A garment embodying the invention is, at least, in part, made of wire and fiber strands associated together and at least in part, covered by an adhering elastomeric coating. In the preferred embodiment the coating is cured or solidified in place.

Advantageously, the wire and fiber strands are associated in a yarn from which the garment is made. For the greatest comfort and flexiblity, the garment is knitted from the yarn. The yarn is formed of a core of one or more strands of wire, advantageously stainless steel wire, and a parallel strand of fiber, preferably synthetic fiber and advantageously polyester fiber, and at least two overwrappings of fiber, preferably synthetic fiber in the form of a thread or strand, of which polyester is most preferred, wound one on top of the other, in opposite directions, about the core.

A garment is knitted from the yarn and coated with a suitable elastomeric material, as by dipping the garment to coat one surface, e.g., the outside surface of a glove, and allowing the coating material to cure in situ, i.e., in place. The coating material must be flexible and have some stretch, be tough, strong, moisture proof, slip resistant, and have good wearing characteristics. Nitrile rubber is particularly suitable. Slip resistance can be improved by incorporating abrasive particles into or onto the coating material.

A garment constructed as described has substantially improved cut-resistance by virtue of the coating. Most surprising is the fact that, while a garment knitted from an aramid and steel wire yarn, and uncoated, has greater cut-resistance than an uncoated garment made from a similarly constructed yarn using other synthetic or natural fibers, such a garment does not maintain that advantage over a garment of yarn using polyester fibers when the garments are coated. In addition, it is difficult to adhere a suitable coating on aramid and polyamide yarn.

Preferably, the garment incorporates a cloth liner that is adhered to the knitted yarn by the coating, which "strikes through" the knitted yarn when it is applied, which is typically accomplished by dipping.

A preferred product and yarn embodying this invention is a protective glove of knitted yarn covered with a coating of elastomeric material cured in place and having a fabric liner bonded in place with the coating, said yarn having a core comprised of four strands of stainless steel wire about 0.003 inch (0.076 mm) in diameter and a parallel core of synthetic polymer fiber having a denier of 800 to 1500, the overall diameter of said core wire being no greater than 0.020 inch (0.51 mm), and said yarn having two strands of polyester fiber having a denier of 210 to 630 wrapped about the core in opposite directions one on top of the other, the total diameter of the yarn being no greater than about 0.050 inch (1.27 mm), said glove being highly cut-resistant, nonabsorbent to dirt, fat, blood and the like, with high slip resistance and good feel to the wearer, and light in weight, stretchable and flexible.

The above and other features and advantages of the invention will become better understood from the detailed description that follows, when considered in connection with the accompanying drawings.
Figure 1 is a front elevational view of a glove embodying the invention;
Figure 2 is a diagrammatic sectional view through a portion of the glove of Figure 1, showing the construction of the material of which the glove is made; and
Figure 3 is a partial elevational view showing the construction of a strand of yarn of which the glove of Figure 1 is made.

A protective garment embodying the present invention is shown in Figure 1 in the form of a safety or protective glove 10 suitable for a variety of uses in handling sharp or rough-edged objects, such as cut metal and glass and for protection from injury from sharp cutting blades and the like. The glove 10 is especially suitable for operators who process meat, where sharp hand knives are used. The invention can also be embodied in other garments, such as wrist guards, protective sleeves, gaiters, and the like.

The glove 10 is made from yarn 12, shown in Figure 3 knitted into a glove shell 13. The preferred glove 10 has a knit cloth liner 14 that is separately made and inserted into the shell 13. An elastomeric coating 16 covers the entire outer surface of the shell, at least up to the edge of a cuff portion 18, where the liner is secured to the knitted glove at the edge of a cuff portion 18 by overcast stitching 20. The coating 16 is preferably applied by dipping the shell 13 and liner together into a suitable coating material in liquid form, removing them from the material and allowing the coating to solidify or cure in place. The coating material strikes through the knitted fabric and secures the liner 14 in place but does not permeate through the liner itself. This is illustrated diagrammatically in Figure 2.

The yarn 12 is comprised of a core 22 formed of a plurality of parallel wire strands 24 extending the length of the yarn and a parallel fiber strand 26, and two fiber strand overwraps 28, 30, helically wound in opposite directions, the strand 28 being wound directly about the core and the strand 30 being an outer strand wrapped about the strand 28 in an opposite helical direction.

The wire strands 24 are flexible and strong and preferably highly corrosion resistant. Stainless steel is a particularly suitable wire strand material, preferably annealed stainless steel wire. While four wire strands are used in the core of the yarn of the preferred embodiment shown, the number of wire strands can vary from 1 to 20 strands, but typically from 2 to 6 strands will be used. The wire strands 24 can range in diameter from 0.001 to 0.010 inch (0.025 to 0.25 mm), the preferred range being from 0.002 to 0.006 inch (0.051 to 0.152 mm) in diameter, and the most preferred size is 0.003 inch (0.076 mm) in diameter. The preferred material is No. 304 stainless steel, fully annealed. Wire diameters smaller than 0.002 inch (0.051 mm) have a shorter advantage over larger diameters. Wire diameters greater than 0.006 inch (0.152 mm) have substantially less flexibility. The total diameter of the single wire strand or the plural wire strands grouped to form the core 22 should not exceed 0.02 inch (0.51 mm), ignoring the fiber strand 26, and preferably will be less than .01 inch (0.25 mm) to faciliate a relatively small overall diameter of the yarn for knitting purposes. While stainless steel is a preferred wire material, especially for garments used in the food industry, where corrosion and food contamination must be avoided and frequent washing is required, other materials are useable in various applications; for example, steel, titanium and other metals may be used that are sufficiently flexible and strong to permit knitting of the yarn and use of the garment.

The parallel fiber strand 26 has high tensile strength, is relatively nonabsorbent, and is a multifilament synthetic polymer fiber, advantageously of a denier of 800 to 1,500. Suitable core fibers include multi-filament fibers of polyester, aramid (aromatic polyamides), and polyamide. The preferred fiber is polyester of about 1000 denier, which avoids the disadvantages of aramid.

A multi-filament strand 26 in the core is advantageous. Multi-filament is continuous rather than spun and slides and/or flows with the other parts of the core during fabrication and subsequent use of an article of apparel produced with the yarn. The high strength multi-filament core strand takes a great deal, if not a major part, of the tensile load to which the yarn is subjected during knitting and use. The filament core strand also appears to increase the flexibility of the core part of the yarn over an all metal core and thus facilitates knitting. Also, a fiber core strand improves the basic quality of the yarn, promoting more even wrapping in the so-called "upwinding" of the yarn. Upwinding is the wrapping of a cover strand about the core. With a wire core, the first winding or overwrap 28 tends to slip longitudinally and a fiber core strand provides much more uniformity in the close spacing or contact between the adjacent turns of a winding about the core. In addition, the presence of a fiber strand in the core acts as a cushion to help the cut-resistance of the wire.

The overwraps 28, 30 are preferably of synthetic polymer fiber, each in the form of a thread or strand made of twisted filaments. Fibers suitable for the overwraps are multi-filament or spun polyester or polyamide. Each strand 26,28 is of a denier of 210 to 630, and in the preferred embodiment is about 440. The wraps 28, 30 are preferably polyester. While aramid and polyamide are advantageous in knitting high strength, cut-resistant gloves that are used in an uncoated form, those materials have been found to be disadvantageous when the glove is to be coated, as in the present invention. Aramid and polyamide are difficult to coat (i.e., to adhere a coating to) and, particularly in the case of aramid, are more expensive than polyester.

While a multi-filament wrap 28, 30 is preferred, it can be a spun filament with a cotton count of from 1 to 60, preferably from 15 to 35. Filament type fibers are preferred over spun fibers because they are stronger and less abrasive in knitting, and they are more resistant to cutting because the tensile strength is greater for any given denier.

Both overwraps 28, 30 are wound with successive turns directly adjacent, as shown. Each is wound in an opposite direction. While two overwraps are preferred, more are possible. It is, however, desirable to have an even number of overwraps for balanced tension. To facilitate use of the yarn in conventional knitting machines and to maintain flexibility in the end product, it is critical that the overall diameter of the yarn be no greater than 0.050 inch (1.27 mm).

The fabric glove portion 13 is knitted rather than formed in other known manners, for flexibility, comfort, seamless construction, and efficiency of manufacture. Preferably it is knitted of a single yarn strand 12. The preferred yarn 12 is comprised of a core 22 of four strands 24 of 304 stainless steel each 0.003 inch (0.076 mm) in diameter and one parallel strand 26 of multi- filament polyester of 1000 denier with two overwraps 28, 30 of polyester multi-filament fiber strands of 440 denier helically wound in opposite directions. The total diameter of the preferred yarn is about 0.025 inch (0.635 mm).

As an alternative to a single yarn, the shell 13 can be of a double yarn (i.e., knitted from two yarns 12, but smaller diameter yarn may then be desired to reduce the weight of the glove). A single yarn knit glove is more desirable in the present invention because the strength and cut resistance of the garment derives more from the metal strands in the core and the coating 16 over the fabric, than from the fiber overwraps 28, 30. Thus, the use of a slightly larger core with four metal strands and, hence, a larger diameter yarn, to form a single yarn knitted glove is more advantageous than using a thinner yarn and a double yarn knitting technique to form the glove. The opposite is true in the case of an uncoated glove in which the overwrap material is of substantially high strength and cut resistance, for example, aramid. A single yarn glove of the present construction is also more flexible and less expensive than a double yarn glove.

A second advantageous construction of the shell 13 utilizes an aramid fiber 26 of 1500 denier in the core and three rather than four stainless wires, each of 0.004 inch (0.10 mm) diameter, but otherwise the same as the preferred embodiment.

The liner 14, which is of cotton or other suitable fabric, such as polyester, provides increased comfort because of its softness and its ability to absorb perspiration. In fabricating the glove 10, a liner 14 is placed over a form to which it tightly conforms. The shell 13 is then placed over the liner and the liner and shell are dipped on the form into elastomeric coating material in liquid form. The material strikes through the knitted yarn of the shell 13, but preferably does not strike through the liner 14. It does however contact the liner 14 and bonds it in place within the shell 13 when the coating material solidifies or cures. The coated shell and adhered liner are removed from the form after curing and the liner and shell are then sewn together at the cuff end by the stitching 20.

Nitrile rubber is the preferred elastomeric coating material, because it is flexible even at low temperatures, stretchable, durable, oil and moisture resistant, tough and cut-resistant, and is relatively slip resistant. The term nitrile rubber includes acrylonitrile rubber, acrylonitrile butadiene rubber, nitrile-silicone rubber, which combines the characteristic properties of silicones with the oil resistance of nitrile rubber, acrylonitrile butadiene rubber, and nitrile butadiene rubber. The preferred nitrile rubber is carboxylated butadiene acrylic nitrile-copolymer latex furnished by Rycold Chemical Co. and includes zinc sulfur butylzymate, clay filler and pigment. Although nitrile rubber is preferred, other elastomers can be used, such as other synthetic polymers (including plastisols and organosols), and natural rubber (polyisoprene). The coating material is solidified or cured in situ, i.e., in place, after the knitted glove 13 is dipped and removed from the bath of the material. Techniques for coating fabric gloves with elastomeric materials are per se known and will be familiar to those skilled in the art.

In the preferred embodiment, the glove 13 is dipped in a manner to apply a continuous, solid (i.e., without exposed yarn) coating over the entire glove surface. Preferably, the coating thickness will be the minimum to provide complete fabric coverage and thereby preserve maximum flexibility and to assure a patterned surface, which is caused by the underlying, coated, shell yarn, which is loosely knitted. The coating thickness is sufficient to make the glove impermeable to liquid and is adequate to provide good wear and, further is sufficiently thick to add substantially to the cut-resistance of the glove. Where rubber nitrile is used as the coating 16, and the glove is of the general construction shown in Figure 1, the dry pick-up weight of the coating material for a medium size glove will typically be about 0.082 pounds (0.0373 kg). The weight of the shell is approximately 0.121 pounds (0.055 kg) and the liner 0.1051 pounds (0.0477 kg), the entire glove being quite light in weight for its strength, cut resistance and other attributes.

After the glove is dipped and removed from the coating material, curing of the nitrile rubber coating is accomplished by heating the coating on the shell to a curing temperature for sufficient time.

Improved slip resistance for gripping can be obtained by increasing the coefficient of friction of the palm and finger portions of the glove by incorporating into or adding an abrasive to the surface of the glove before the coating material is cured. Such a material may include pumice, by way of example. In addition, or alternatively, natural rubber or flock can be applied to the surface and/or a pattern can be impressed upon the glove in the palm and finger portions.

As compared with known aramid fiber gloves as disclosed in U.S. Patent No. 4,004,295, U.S. Patent Application Serial No. 99,092 filed November 30, 1979, and U.S. Patent Application Serial No. 891,611 filed March 30, 1978, the present glove represents a different approach to cut resistance and provides the many advantages of the coating material. Aramid, for example, requires a chemical bond to facilitate coating and agents that provide such a bond are typically dangerous in food and would limit the uses of the glove. Also, the abrasiveness of aramid within the coating material causes deterioration of the yarn. Furthermore, use of a greater number of strands of wire 24 is made possible by using polyester rather than aramid in knitted products and especially knitted products that require flexibility, such as gloves. Because aramid essentially does not stretch, a yarn that uses four or more strands of wire becomes much too rigid for knitting and for most uses when aramid is used as a core and wrapping. With the present construction and the use of more stretchable polyester, additional wire of significant diameter imparts high cut resistance without unacceptable rigidity. In terms of strength, the flexibility and stretch of the core fibre, when the yarn is subjected to strain, allows the tensile strength of the increased quantity of steel to be utilized in resisting cutting. The flexibility of the yarn also allows use of an elastomeric coating without exceeding acceptable stiffness in the final product.

From the above, it will be apparent that a new and improved protective garments is provided, that is liquid proof and not absorbent to dirt, fats, oil, blood and other fluids, that is cut resistant, abrasion resistant, light in weight, flexible and comfortable to wear, and that is neither self- abrasive not abrasive to other objects or clothing that it contacts (unless the coating is purposefully modified to increase friction). It also provides protection from heat. When the garment is in the form of a glove, it has a good feel and grip. While the glove industry has tradionally used layers of material to provide cut resistance and protection, the present garment provides an integral construction that is highly cut-resistant. Its combined features meet a wide range of needs.

## Claims

1. A flexible protective garment, at least part of which is knit from a yarn having a core of wire and fiber, with a protective coating, characterized by a knit shell (13) made of fiber and metal wire, a knit fabric liner (14) separately formed and located within the shell, and an elastomeric coating (16) adhered to and permeating the shell, solidified or cured in place, and adhered to but not penetrating through the liner, securing the liner in place.

2. The protective garment as set forth in Claim 1 characterized in that at least a part of said knit shell (13) is made of yarn (12) comprising a core (23) having one or more strands of flexible wire (24) and a covering of one or more fiber strands (28, 30).

3. The protective garment as set forth in Claim 1 characterized in that said core (22) includes a fiber strand (26) extending parallel to the one or more strands of wire (24) and the one or more fiber strands (28, 30) are helically wrapped about the core.

4. The protective garment as set forth in Claim 2 or 3 characterized in that the core (22) includes to to twenty strands of annealed stainless steel wire each having a diameter of 0.025 to 0.25 millimeter.

5. The protective garment as set forth in any of the preceding claims characterized in that the total diameter of the yarn (12) is no greater than 1.27 millimeter.

6. The protective garment as set forth in any of Claims 2-5 characterized in that it is at least in part tubular in shape and at least in part made from yarn (12) comprised of a core (22) having 2 to 6 strands (24) of annealed stainless steel wire 0.051 to 0.15 millimeter in diameter and a parallel synthetic polymer fiber strand (26) having a denier of 800 to 1500, the overall diameter of the wire strands being no greater than 0.51 millimeter, and at least two strands (28, 30) of polyester fiber having a denier of 210 to 630 wrapped about the core in opposite directions one on top of the other.

7. The protective garment as set forth in Claim 6 characterized in that the core (22) has 4 strands (24) of stainless steel wire each 0.076 millimeter in diameter and the garment is a safety glove.

8. The protective garment as set forth in Claims 2-7 characterized in that the fiber strands (24) are either polyamide or polyester fibers.

9. protective garment as set forth in any of the preceding claims wherein the elastomeric coating (16) is nitrile rubber.

## Patentansprüche

1. Flexibles Schutzbekleidungsstück, das mindestens zum Teil aus einer Maschenware aus einem Garn besteht, das einen Kern aus Draht und Fasermaterial besitzt un mit einem Schutz- überzug versehen ist, gekennzeichnet durch eine gemaschte Hülle (13) aus Fasermaterial und Metalldraht, ein aus einer Maschenware bestehendes Futter (14), das getrennt von der Hülle hergestellt und in ihr angeordnet ist, und einen elastomeren Überzug (16), der an der Hülle haftet und sie durchdringt, in situ erstarrt oder erhärtet ist und an dem Futter haftet, aber es nicht durchdringt und der das Futter festhält.

2. Schutzbekleidungsstück nach Anspruch 1, dadurch gekennzeichnet, daß mindestens ein Teil der gemaschten Hülle (13) aus einem Garn (12) besteht, das einen Kern (23) besitzt, der einen oder mehrere Litzen auf flexiblem Draht (24) besitzt, wobei das Garn ferner ein oder mehrere Faserbündel (28, 30) besitzt.

3. Schutzbekleidungsstück nach Anspruch 1, dadurch gekennzeichnet, daß der Kern (22) ein Faserbündel (26) besitzt, das zu dem einen oder den mehreren Faserbündel (24) parallel ist, und daß das eine oder die mehreren Faserbündel (28, 30) wendelförmig um den Kern gewickelt sind.

4. Schutzbekleidungsstück nach Anspruch , 2 oder 3, dadurch gekennzeichnet, daß der Kern (22) zwei bis zwanzig Bündel aus geglühtem nichtrostenden Stahldraht mit einem Durchmesser von je 0,025 bis 0,25 mm enthält.

5. Schutzbekleidungsstück nach einem der vorhergehenden Ansprüche, dadurch gekennzeichnet, daß der Gesamtdurchmesser des Garns (12) nicht größer ist als 1,27 mm.

6. Schutzbekleidungsstück nach einem der Ansprüche 2 bis 5, dadurch gekennzeichnet, daß es mindestens teilweise schlauchförmig ist und mindestens zum Teil aus einem Garn (12) besteht, das einen Kern (22) mit zwei bis sechs Bündeln (24) aus geglühtem nichtrostendem Stahldraht mit einem Durchmesser von 0,051 bis 0,15 mm und mit einem Bündel (26) aus parallelen synthetischen Polymerfasern mit einem Titer von 800 bis 1500 Denier besteht, wobei der Gesamtdurchmesser der Drahtbündel nicht größer ist als 0,51 mm und mindestens zwei Bündel (28, 30) aus Polyesterfasern mit einem Titer von 210 bis 630 Denier um den Kern in entgegengesetzten Richtungen übereinandergewickelt sind.

7. Schutzbekleidungsstück nach Anspruch 6, dadurch gekennzeichnet, daß der Kern (22) vier Bündel (24) aus nichtrostendem Stgahldraht mit einem Durchmesser von je 0,076 mm besitzt und das Bekleidungsstück ein Sicherheitshandschuh ist.

8. Schutzbekleidungsstück nach den Ansprüchen 2 bis 7, dadurch gekennzeichnet, daß die Faserbündel (24) aus Polyamid- oder Polyesterfasern bestehen.

9. Schutzbekleidungsstück nach einem der vorhergehenden Ansprüche, dadurch gekennzeichnet, daß der elastomere Überzug (16) aus Nitrilkautschuk besteht.

## Revendications

1. Vêtement souple de protection, dont au moins une partie est tricotée à partir d'un fil comportant une âme en fil métallique et fibres et muni d'un revêtement protecteur, caractérisé par une coque tricotée (13) réalisée en fibres et en fil métallique, par un fourreau (14) en tissu de fil formé séparément et mis en place à l'intérieur de la coque, et par un revêtement élastomère (15) amené en adhérence avec et infiltrant la coque, solidifié ou durci en place, et amené en adhérence avec, mais ne pénétrant pas dans le fourreau, et fixant le fourreau en place.

2. Vêtement de protection selon la revendication 1, caractérisé en ce qu'au moins une partie de la coque tricotée (13) est constituée de fil (12) comprenant une âme (23) comportant un ou plusieurs brins en fil métallique souple (24) et un recouvrement d'un ou de plusieurs brins en fibres (28, 30).

3. Vêtement de protection selon la revendication 1, caractérisé en ce que ladite âme (22) comprend un brin en fibres (26) s'étendant parallèlement au(x) brin(s) en fil métallique (24) et en ce que le ou les brins en fibres (28, 30) sont enroulés en hélice autour de l'âme.

4. Vêtement de protection selon la revendication 2 ou 3, caractérisé en ce que l'âme (22) comprend de deux à vingt brins de fil d'acier inoxydable recuit ayant chacun un diamètre compris entre 0,025 et 0,25 mm.

5. Vêtement de protection selon l'une des revendications précédentes, caractérisé en ce que le diamètre total du fil (12) ne dépasse pas 1,27 mm.

6. Vêtement de protection selon l'une des revendications 2 à 5, caractérisé en ce qu'il est au moins en partie de forme tubulaire et au moins en partie réalisé à partir d'un fil (12) constitué par une âme (22) comportant de 2 à 6 brins (24) de fil d'acier inoxydable recuit d'un diamètre de 0,051 à 0,15 mm et un brin parallèle (26) en fibres polymères synthétiques de 800 à 1500 deniers, le diamètre global des brins en fil métallique ne dépassant pas 0,51 mm, et par au moins deux brins (28, 30) en fibres de polyester de 210 à 630 deniers enroulés autour de l'âme dans des sens opposés l'un par-dessus l'autre.

7. Vêtement de protection selon la revendication 6, caractérisé en ce que l'âme (22) comporte quatre brins (24) en fil d'acier inoxydable ayant chacun un diamètre de 0,076 mm et en ce que le vêtement est un gant de sécurité.

8. Vêtement de protection selon l'une des revendications 2 à 7, caractérisé en ce que les brins en fibres (24) sont en fibres de polyamide ou de polyester.

9. Vêtement de protection selon l'une des revendications précédentes, dans lequel le revêtement élastomère (16) est un caoutchouc de nitrile.
